

T. B. STONE.  
Grinding and Polishing Implement.

No. 223,771.

Patented Jan. 20, 1880.

Fig. 1.



Fig. 2.



Fig. 3.

Witnesses

Chas. A. Coole,  
John Lockie

Inventor

Tucker B. Stone  
Per W<sup>m</sup> R. Singleton  
Atty.

# UNITED STATES PATENT OFFICE.

TUCKER B. STONE, OF ST. LOUIS, MISSOURI.

## GRINDING AND POLISHING IMPLEMENT.

SPECIFICATION forming part of Letters Patent No. 223,771, dated January 20, 1880.

Application filed September 19, 1879.

*To all whom it may concern:*

Be it known that I, TUCKER B. STONE, of St. Louis, in the county of St. Louis and State of Missouri, have invented certain Improvements in Grinding and Polishing Implements, of which the following is a specification.

This invention relates to tools for grinding and polishing; and it consists in the combination of certain materials found in nature, 10 which, after due process, are to be molded into the shapes required, and afterward properly hardened in a furnace, all of which will be hereinafter more fully described, and set forth in the claim.

15 The principal substance used in the following compound is known in mineralogy as "itacolumite," which is commonly called "flexible sandstone." Its analysis shows the following ingredients and their proportions, viz: bort, 20 sixty-seven per cent.; silica, twenty-eight per cent.; mica, two per cent.; and water of crystallization, three per cent.

I take the following substances, which may be broken up in small pieces, so that they will 25 be readily fused, viz: one part of feldspar, one part of saltpeter, three parts of borax, two parts of sand, and three parts of soda-ash. These ingredients are to be mixed thoroughly in a crucible and melted, so as to form one 30 mass, after which the mass is allowed to cool, and then pulverized to the degree of fineness required for the grit of the tool to be used for grinding or polishing, to make the coarse

or very fine polishing-tool. This pulverized material is then to be mixed with eighty parts 35 of the itacolumite, which had been previously reduced to a powder similar in fineness to that of the other. When these have been thoroughly incorporated the mass is to be moistened with water sufficiently to permit it to be tamped 40 in molds of the proper form, such as shown in the drawings, Figures 1, 2, and 3, and such pressure is to be applied as may be necessary to compress the mass to the firmness which may be requisite. The material thus molded is 45 then placed in a suitable furnace until the tool is sufficiently baked. After cooling the same it is ready for use. This material can be molded into any shape for polishing, grinding, or reducing surfaces, plain or molded. 50

Grinding-stones may be made of any size or hardness, and of all grades of fine or coarse, as the work may require.

I claim—

Implement for reducing, grinding, and polishing surfaces, composed of a mixture of the following materials, and of approximate proportions as follows: one part each of feldspar and saltpeter, two parts of sand, and three parts each of borax and soda-ash, and eighty 55 parts of pulverized itacolumite, substantially as and for the purpose described.

TUCKER B. STONE.

Witnesses:

F. S. MACK,  
R. B. WASHINGTON, Jr.